

# United States Patent [19]

Anderson, Jr. et al.

[11] 3,753,701

[45] Aug. 21, 1973

[54] **REFRACTORY METAL ALLOYS FOR USE IN OXIDATION ENVIRONMENTS**

[75] Inventors: Wallace T. Anderson, Jr., Huntington Beach; Ralph A. Mendelson, Westminster, both of Calif.

[73] Assignee: TRW Inc., Redondo Beach, Calif.

[22] Filed: Dec. 30, 1971

[21] Appl. No.: 214,352

[52] U.S. Cl. .... 75/175.5

[51] Int. Cl. .... C22c 15/00

[58] Field of Search..... 75/174, 175.5

[56] **References Cited**

UNITED STATES PATENTS

2,940,845 6/1960 Jaffee et al. .... 75/175.5 X  
3,028,236 4/1962 Wlodek et al. .... 75/174

FOREIGN PATENTS OR APPLICATIONS

782,564 9/1957 Great Britain ..... 75/175.5  
241,676 7/1969 U.S.S.R. ..... 75/175.5

Primary Examiner—Charles N. Lovell

Attorney—Daniel T. Anderson, Willie Krawitz et al.

[57] **ABSTRACT**

A refractory metal alloy comprising principally columbium and titanium, with lesser amounts of beryllium, chromium, silicon and yttrium provides excellent resistance to air oxidation at high temperature.

The broad composition range is as follows:

Columbium 32.5–46 percent; Titanium 50.5–57.5 percent; Beryllium 0–8 percent; Chromium 2.15–2.6 percent; Silicon 0–8 percent; and Yttrium 0–0.1 percent; all parts by weight.

2 Claims, 4 Drawing Figures

OXIDATION IN AIR OF A PRIOR ART ALLOY (45at. % Nb–50at. % Zr–5at. % Ti) at 1200°C & THE PRESENT ALLOY AT 1300°



PATENTED AUG 21 1973

3,753,701

SHEET 1 OF 2

OXIDATION IN AIR OF A PRIOR ART ALLOY (45at. % Nb-50at. % Zr-5at. % Ti) at 1200°C & THE PRESENT ALLOY AT 1300°



PATENTED AUG 21 1973

3,753,701

SHEET 2 OF 2



Fig. 2



Fig. 4

## REFRACTORY METAL ALLOYS FOR USE IN OXIDATION ENVIRONMENTS

### BACKGROUND OF THE INVENTION

This invention relates to new and improved refractory metal alloys. More specifically, this invention relates to refractory metal alloys having columbium and titanium as the principal alloy ingredients: beryllium, chromium, silicon and yttrium are minor constituents.

Refractory alloys have been employed as castings, forgings, etc., at high temperatures. Typical examples of refractory alloys are found in U.S. Pat. Nos. 3,086,859; 2,940,845; 2,991,197; 2,880,088; 2,819,960; 2,754,204; and 3,368,881.

However, their use at high temperature in an oxidizing environment is limited since the amount of oxidation continues with increasing time which eventually results in failure of the alloy as it becomes converted into an oxide.

It is, therefore, an object of the present invention to provide a refractory alloy which may be employed as castings, forgings, etc., in a high temperature, oxidizing environment such as air.

Other objects will be disclosed from the description and graphs to follow.

According to the invention, the broad range of the components in the refractory alloy is as follows:

Columbium 32.5-46 percent; Titanium 50.5-57.5 percent; Beryllium 0-8 percent; Chromium 2.15-2.6 percent; Silicon 0-8 percent; and Yttrium 0-0.1 percent; all parts by weight.

A narrower range of components is as follows:

Columbium 33.5-44.5 percent; Titanium 52-56 percent; Beryllium 0-7.5 percent; Chromium 2.2-2.5 percent; Silicon 0-7 percent, and Yttrium 0-0.1 percent; all parts by weight.

Specific alloy compositions of this invention are:

| Composition | Columbium | Titanium | Beryllium | Chromium | Silicon | Yttrium |
|-------------|-----------|----------|-----------|----------|---------|---------|
| 1.          | 44.5      | 52.2     | 1.0       | 2.2      | 0       | 0.1     |
| 2.          | 44.4      | 52.2     | 0         | 2.2      | 1.1     | 0.1     |
| 3.          | 43.4      | 52.2     | 1.0       | 2.2      | 1.1     | 0.1     |
| 4.          | 42.4      | 52.2     | 2.0       | 2.2      | 1.1     | 0.1     |
| 5.          | 41.4      | 52.2     | 1.0       | 2.2      | 3.1     | 0.1     |
| 6.          | 40.9      | 52.2     | 3.5       | 2.2      | 1.1     | 0.1     |
| 7.          | 39.4      | 52.2     | 1.0       | 2.2      | 5.1     | 0.1     |
| 8.          | 38.0      | 52.2     | 7.5       | 2.2      | 0       | 0.1     |
| 9.          | 37.4      | 52.2     | 1.0       | 2.2      | 7.1     | 0.1     |
| 10.         | 36.9      | 52.2     | 7.5       | 2.2      | 1.1     | 0.1     |
| 11.         | 33.8      | 55.9     | 1.0       | 2.5      | 6.8     | 0       |

The oxidation resistance of the present alloys was tested by exposure to air at temperatures between 50 1,100° C and 1,300° C. The weight gain of the alloys, which is considered to indicate the extent of oxidation,

was measured as a function of the exposure time.

In the drawings, FIGS. 1-4 are graphs showing the relationship between exposure time and weight gain (due to oxidation) of the alloy compositions at various oxidation temperatures in air.

FIG. 1 shows a comparison of the oxidation resistance in air of alloy composition 9 with that of a typical prior art refractory metal alloy having the composition 45 at. % Nb; 50 at. % Zr; 5 at. % Ti. It will be observed that the curve of composition 9 at 1,300° C is well below that of the prior art alloy at 1,200° C; this represents a significant improvement in oxidation resistance.

As shown in FIG. 2, compositions 2, 4, 5, and 9 show significant improvement (about twice the oxidation resistance) over the prior art alloy when exposed to air at 1,200° C.

In FIG. 3, compositions 4, 5, and 7 are significantly improved over the prior art composition at 1,300° C. Composition 2 was significantly more oxidized at 1,300° C than the prior art alloy composition.

In FIG. 4, compositions 1, 3, 8, and 6 performed quite well at 1,100° C and showed no tendency to rapid oxidation.

Hence, the alloy compositions of this invention are markedly resistant to oxidation at high temperatures and show little tendency to rapidly accelerate in oxidation as compared to the prior art alloy. This renders them well suited for use as castings, forgings, etc., in air at high temperatures.

We claim:

1. A refractory alloy composition consisting of: Columbium 32.5-46 percent; Titanium 50.5-57.5 percent; Beryllium 0-8 percent; Chromium 2.15-2.6 percent; Silicon 0-8 percent; and Yttrium 0-0.1 percent; all parts by weight.

2. A refractory alloy composition consisting of:

Columbium 33.5-44.5 percent; Titanium 52-56 percent; Beryllium 0-7.5 percent; Chromium 2.2-2.5 percent; Silicon 0-7 percent; and Yttrium 0-0.1 percent; all parts by weight.

\* \* \* \* \*